

H. V. LOSS.

METHOD OF HEATING BARS OR BILLETS PREPARATORY TO FORGING.

APPLICATION FILED DEC. 13, 1911.

1,084,156.

Patented Jan. 13, 1914.

*Fig. 1.*



*Fig. 2.*



*Fig. 3.*

WITNESSES

*E. J. Gamble*

*J. D. Grapp*

BY

*Chas A. Carter*

ATTORNEY

*Henrik V. Loss*

# UNITED STATES PATENT OFFICE.

HENRIK V. LOSS, OF PHILADELPHIA, PENNSYLVANIA.

## METHOD OF HEATING BARS OR BILLETS PREPARATORY TO FORGING.

1,084,156.

Specification of Letters Patent.

Patented Jan. 13, 1914.

Application filed December 13, 1911. Serial No. 665,439.

To all whom it may concern:

Be it known that I, HENRIK V. Loss, a citizen of the United States, and a resident of the city and county of Philadelphia, State 5 of Pennsylvania, have invented certain new and useful Improvements in Methods of Heating Bars or Billets Preparatory to Forging, of which the following is a specification.

10 My invention relates to improvements in the heating of metal bars or billets preparatory to forging them in dies, and more particularly to improvements in method of heating bars or billets preparatory to forging them in dies into axles for service with rolling stock of railways.

In Letters Patent of the United States No. 812,856, issued to me upon February 20, 1906, a method for forging axles is disclosed. 20 Briefly this method consists in placing the central part of the bar or billet to be forged between longitudinally separable central dies, gripping its ends between longitudinally separable movable dies, moving the 25 latter dies toward the central dies so as to cause the metal to be pushed inward to fill the central die and completing the forging with header dies which are moved toward the movable dies. In this process it is absolutely necessary in order to produce a perfect forging that the central die be completely filled with metal and as this die has the form of two truncated cones the smaller diameters of which meet at its middle and 35 the bases of which are at, or substantially at, its outer ends it is desirable that the bar or billet be so heated that when it is upset by the inward movement of the movable dies that the first upsetting will take place within 40 the central die, commencing at or about the middle and gradually moving forward, and that after this die is filled the upsetting of the outer part, approximately that part from the inner end of the wheel seat to the outer 45 end of the axle, will be accomplished.

If the bar or billet be evenly heated throughout its entire length it would be just as likely as not to upset first in the movable dies, or to be bent at the exposed portion between the central and movable dies. In such an event the upsetting would probably not result in completely filling the central die and an imperfect forging would result.

In order to insure the proper sequence in 50 the upsetting of the bar or billet, according to my method of forging axles from the

same, I purpose to heat the whole bar or billet to a forging temperature but to heat the central part hotter than the ends so that this part may be the softest and the first to 60 upset when the bar or billet is pushed inward by the movable dies.

In the accompanying drawing Figure 1 represents a side elevation of a bar or billet before upsetting; Fig. 2, a side elevation of 65 the same after being upset according to the method disclosed in my patent above referred to, Fig. 3 a longitudinal sectional elevation through a set of axle forging dies in which my process for forging may be carried out.

Referring to Fig. 3; 1 and 2 are upper and lower longitudinally separable central dies. 3-4 longitudinally separable movable dies. 5 header dies. Dies substantially 75 similar to these were shown in my patent above referred to. The outer parts of the bar or billet to be upset are grasped by the movable dies 3-4 and at its middle preferably, but not necessarily, by the stationary 80 dies 1-2. The movable dies are now moved toward one another and the bar or billet is upset and fills the interior of the central dies which correspond in shape to that of the middle part of the axle. The middle 85 part of the axle having been formed the header dies 5 are moved in to upset the ends to form the extreme ends of the axle.

Preparatory to placing the bar or billet in the dies in which it is to be forged into 90 an axle I heat its central part, say between the inner ends of the parts *a* which are to form the wheel seats, to a greater degree than the parts that lie outside of these inner ends, consequently the center part of the 95 bar or billet is the softest and first responds to the upsetting action of the dies gradually and completely filling the central die, thus forming the part *x-y* of the axle, before the upsetting action takes place outside of this 100 part.

In order to completely fill the central dies the upsetting should commence at a point midway between the ends, at which point the diameter of the axle is the smallest. I 105 would, without desiring to limit myself strictly thereto, prefer in most cases to heat that part of the bar or billet which is midway of its ends to the maximum heat, to gradually reduce this heat toward the points 110 which are to form the wheel seats and from this latter point outward to still further de-

crease the heat thus insuring the upsetting of the bar or billet first at its middle and then gradually outward to its ends.

It will be observed that I heat all parts 5 of the bar or billet simultaneously by radiation from a furnace and to a forging temperature throughout its entire length, heating, however, the part that is to be first upset to a greater degree than the parts that 10 are to be subsequently upset so that there will be no question as to the metal filling all parts of the dies which form the finished product.

Having thus described my invention I 15 claim as new and desire to secure by Letters Patent:—

1. The described process for preparing a bar or billet for the dies of a longitudinally operating upsetting machine which consists

in heating by radiation the bar or billet 20 throughout its entire length to a forging heat and the part intermediate of its ends to a greater degree than its ends.

2. The described method for preparing a bar or billet for longitudinal upsetting in 25 an axle forging machine, which consists in unequally heating by radiation the bar or billet to a forging temperature throughout its entire length, the central part of the bar being heated to the maximum degree, this 30 heat being properly decreased in those parts of the bar that are to form the wheel seats, journals and collars.

HENRIK V. LOSS.

Witnesses:

CHARLES A. RUTTER,  
CHARLES HERNION.